

Dec. 13, 1966

R. G. FLOWERS ET AL

3,291,639

METHOD OF INSULATING ELECTRICAL CONDUCTORS

Filed Feb. 25, 1963

5 Sheets-Sheet 1



INVENTORS,  
Ralph G. Flowers,  
Thomas L. Sherer,  
by Francis X. Doyle  
Their Attorney.

Dec. 13, 1966

R. G. FLOWERS ET AL

3,291,639

METHOD OF INSULATING ELECTRICAL CONDUCTORS

Filed Feb. 25, 1963

3 Sheets-Sheet 2

Fig. 4.



Fig. 5.



Inventors,  
Ralph G. Flowers,  
Thomas L. Sherer,  
by Francis K. Doyle  
Their Attorney.

Dec. 13, 1966

R. G. FLOWERS ET AL

3,291,639

METHOD OF INSULATING ELECTRICAL CONDUCTORS

Filed Feb. 25, 1963

3 Sheets-Sheet 3



Inventors,  
Ralph G. Flowers,  
Thomas L. Sherer,  
by *Francie K. Doyle*  
Their Attorney.

## 1

3,291,639

## METHOD OF INSULATING ELECTRICAL CONDUCTORS

Ralph G. Flowers, Pittsfield, and Thomas L. Sherer, Richmond, Mass., assignors to General Electric Company, a corporation of New York

Filed Feb. 25, 1963, Ser. No. 260,641  
4 Claims. (Cl. 117—232)

This invention relates to insulating electrical conductors and more particularly to a novel process of insulating electrical conductors and the conductors insulated by such process.

It is well known to those skilled in the electrical insulating art to apply a type of enamel film insulation to electrical conductors, such as wires and the like. In general, the electrical conductor is coated in a "wire mill" in which an elongated wire is taken from a supply reel and passed continuously through a bath of insulating coating liquid. The wire with the coating material adhering thereto is then passed through a drying or curing oven where the insulating coating is hardened or cured. The wire is then passed through the insulating bath and the drying oven in repeated stages until a coating of the desired thickness has been built up on the electrical conductor. The coated insulated wire is then usually wound on a take-up reel for storage purposes until needed.

In coating electrical conductors in this manner, the curing of the insulating enamel material results in a chemical reaction in which one of the constituents of the enamel reacts with another constituent to form a cross linked, tough, flexible film insulation. In this process water and/or other volatile by-products are evolved. These by-products must be substantially eliminated in order to provide a good electrical insulation. It is the usual practice to try to eliminate these volatile by-products by use of the drying oven which provides a high temperature cure to the various layers of film insulation.

In order to substantially eliminate these volatile by-products during the curing of the film insulation, and to produce a good electrical insulation, excessive temperatures are required which have an undesirable side effect. This undesirable side effect is that these high curing temperatures have an adverse effect on the physical properties of the film insulation. In general, it is found that the film insulation tends to become embrittled when subjected to the high curing temperatures in the normal curing oven, thereby rendering the insulated electrical conductor subject to damage from winding or abrasive action. Thus in the present-day insulating art, the temperature of the drying oven and the time of passage of the coated electrical conductor therethrough is set as a compromise between the substantial elimination of the volatile by-products to provide optimum electrical properties, and the physical degradation of the insulating film which can be accepted for insulated electrical conductors under the particular circumstances of intended use for the particular conductor.

It has been recently discovered that the embrittlement of the film insulation is in part caused by the combination of the oxygen with the curing film at the curing temperature. It has further been discovered that if the detrimental effects of the oxygen can be eliminated or reduced, that a more optimum chemical cure to obtain desired electrical properties can be obtained without any adverse effects on the physical properties of the film. A further discovery has been made in that insulated film on wire that has previously been cured in the normal manner may have its electrical properties substantially improved by a further curing in which the detrimental effects of oxygen on curing are eliminated.

## 2

It is, therefore, one object of this invention to provide an improved method of insulating electrical conductors.

It is a further object of this invention to provide an improved film insulated electrical conductor.

5 A further object of this invention is to provide a new curing method for film insulation on electrical conductors.

A further object of this invention is to provide an additional curing method for previously cured film-insulated electrical conductors.

10 A further object of this invention is to provide an improved film insulation on electrical conductors by subjecting such conductors to a second improved curing.

In carrying out this invention in one form thereof, an improved film-insulated electrical conductor is provided in 15 which the film insulation is cured in a nonoxidizing medium. In another form of the invention a cured film-insulated electrical conductor is subjected to a further cure in a nonoxidizing medium.

The invention which is desired to be protected will be 20 clearly pointed out and distinctly claimed in the claims appended hereto. However, it is believed that this invention and the manner of carrying it out, as well as the manner in which its various objects and advantages are obtained, together with other objects and advantages thereof will be more clearly understood by reference to the following detailed description of various preferred embodiments thereof, particularly when taken in connection with the accompanying drawings, in which:

FIGURE 1 is an elevation view partly in section showing 30 one form of this invention applied to a continuous coating apparatus;

FIGURE 2 is an elevation view partly in section showing 35 one form of apparatus according to this invention for providing a second cure to previously cured film-insulated electrical conductors;

FIGURE 2a is a partial sectional view showing a modification which may be used with the apparatus of either 40 FIGURE 1 or FIGURE 2;

FIGURE 3 is a group of curves showing the dissipation 45 factor of cured polyvinyl formal coated electrical conductors at various temperatures, and illustrating the improvement which may be obtained by means of this invention;

FIGURE 4 is another group of curves showing the dissipation 50 factor of cured polyvinyl formal coated electrical conductors at various temperatures pointing out the improvements which may be obtained by one form of this invention;

FIGURE 5 is a group of curves of an epoxy enamel 55 film insulation cured on an electrical conductor showing the improvements which may be obtained by means of one form of this invention;

FIGURE 6 is a group of curves of a polyester type 60 enamel film insulation cured on an electrical conductor to show the improvements which may be obtained by means of one form of this invention; and

FIGURE 7 is a group of curves showing the improved 65 aging characteristics of a polyvinyl formal enamel coated insulated electrical conductor when cured according to one form of this invention.

As earlier noted, it has been discovered that the electrical properties of film insulation on electrical conductors can be substantially improved without detrimental effects to their physical properties when the film-coated wire is cured in a nonoxidizing atmosphere or medium.

65 FIGURE 1 shows one form of coating apparatus which may be used to carry out the method of this invention. A wire coating mill is shown in FIG. 1 for coating continuously moving electrical conductors. As shown in FIG. 1, the wire mill comprises a base member 10 having a quantity of a suitable insulating coating liquid 12 therein, and a baking or drying oven 14 mounted on top

of the base member 10. An electrical conductor 16, to be coated in the wire mill, is wound upon a supply reel 18 and is led from such supply reel through a guide sheave 20 mounted in the base member 10 within the liquid insulating coating 12, in the manner shown. Wire 16 is led around the guide sheave 20 where it is provided with the coating material which adheres thereto and then passes through a die device 22, such as is well known to those skilled in the art, and extends up through the drying oven 14 where it passes around a second guide sheave 24. The wire 16 is then returned to the base member 10 back through the insulating liquid 12 about a second guide sheave, behind guide sheave 20, where a second coating of the insulating liquid is applied thereto, again, through the drying oven and around a further guide sheave 24 at the top. The wire 16 passes through the coating and drying apparatus in repeated stages until a coating of the desired thickness is built up on wire 16. The coated wire is finally conducted to a take-up reel 26.

The novel feature of the wire mill disclosed in FIG. 1 is in the drying oven 14. As shown, the drying oven 14 comprises refractory side walls 28 and 30. Each of the side walls is provided with electrical heating means 32, as is well understood by those skilled in this art. Similar end walls (not shown) are also provided. The drying oven is securely attached to the base member 10 of the wiring mill. As is shown in the drawing, a substantially air-tight sealing member 34 is provided over the open portion of the base member 10 contacting both the base member and side 30 of the drying oven. Sealing member 34 is provided with openings 36 and 38 therein to allow the wire 16, as it passes from the take-up reel 18 and from the guide sheave 24, to enter the base member 10. As will be understood, each of openings 36 and 38 are provided with sealing means, such as rubber gaskets or the like 37, 39, so as to prevent entry of air into the drying oven 14. The top of the drying oven is similarly provided with a cap member 40. The cap member 40 is also provided with openings 42 therein for the passage of wire 16 therethrough. Each of openings 42 is similarly provided with sealing means in the form of rubber gaskets or the like, 43, to prevent the entry of air therein. Member 34 is provided with an opening therein, indicated at 44, and a neck member 46 extends from the opening. The neck member 46 leads from the sealing member 34 and the drying oven 14 to a device 48 which may be either a vacuum pump or which may be a device for providing a nonoxidizing atmosphere, such as carbon dioxide, nitrogen or other gas to the interior of the drying oven 14. Member 34 may be provided with an inwardly extending shelf member 33 having openings 35 therein, if desired. Shelf member 33 will help to prevent liquid coating material 12 from being drawn into device 48, when it is a vacuum pump.

As is well understood, by means of device 48, where device 48 is a vacuum pump, when the drying oven is being used the vacuum pump may be operated to substantially evacuate the interior of the drying oven 14 to thereby provide a substantially nonoxidizing atmosphere in the form of a vacuum. Of course, the drying oven 14 must be designed such that a vacuum may be drawn without damage to the oven. However, it is also possible, as will be understood, to provide an atmosphere of either carbon dioxide, nitrogen, or other non-oxidizing gas within the drying oven 14 where the device 48 will be a storage tank of either carbon dioxide, nitrogen, or other gas which will be admitted under pressure into the interior of the drying oven 14. As will be understood, whichever is utilized, the interior of the drying oven will be substantially a nonoxidizing atmosphere for providing curing of the coated wire 16 extending through the drying oven. Thus it will be apparent, that by means of a wire mill, similar to that disclosed in FIG. 1 of the drawing, it is possible to coat electrical conductors with an insulating liquid and to cure such

insulating liquid in a nonoxidizing atmosphere to thereby substantially eliminate the volatile by-products of such coating without deteriorating or adversely affecting the physical properties of such coating.

Referring now to FIG. 2 of the drawing there is shown therein a curing oven substantially similar to that shown in FIG. 1, wherein film-insulated electrical conductors may be provided with a second cure, hereinafter called "post-cure" or "post-cured," to substantially improve the electrical insulating properties of the film insulation without adversely affecting the physical properties of the film insulation. As is shown in FIG. 2, a drying oven 14' is provided having opposite refractory side walls 28', 30' and electrical heating means 32' mounted in such refractory side walls, in the same manner as indicated with reference to FIG. 1. Similar end walls (not shown) are also provided. The top of the drying oven is provided with a top sealing member 50 having openings 42' therein, in the same manner as set forth with reference to FIG. 1. As will be understood, member 50 is sealed in an air-tight manner to the top of drying oven 14'. The lower end of the drying oven is provided with a base member 52 substantially sealing the bottom of the drying oven and having openings 54 therein. Each 54 is provided with sealing means, in the form of rubber gaskets or the like 55.

In this apparatus, where it is desired to post-cure the previously cured film-insulated electrical conductors, each conductor 16' is mounted on a supply reel 18' and the conductor 16' is led from such supply reel through a guide sheave 20' through openings 54 and rubber seals 55 and into the drying oven 14'. The insulated wire 16' comes out of the drying oven through opening 42' in the cap member 40 around a guide sheave 24' and onto a take-up reel 26'. As will be understood, in this device it is only necessary that the wire 16' be passed through the drying oven 14' once, inasmuch as there is no requirement in this drying oven to cure separate insulating coatings applied to the conductor, in the manner of the wire mill of FIG. 1. Further, as will be understood, the passage of the conductor through the drying oven 14' may be set at the particular desired time according to the temperature of the oven and the type of electrical insulation film on the wire 16' to provide the desired cure of such enamel film insulation, as will be more clearly specified hereinafter. Further, in a manner similar to that shown with reference to FIG. 1, an opening 44' is provided in the sealing member 50 of the drying oven, and the opening 44' has provided therein a neck member 46'. Neck member 46' goes to a device 48' which may either be a vacuum pump or a supply of carbon dioxide, nitrogen, or other gas as hereinbefore more fully discussed with reference to FIG. 1.

Sealing member 50 may also be provided with a second neck member 58 extending to an open chamber 60. As will be understood, when carbon dioxide, nitrogen or similar nonoxidizing gas is introduced into member 50 and oven 14' under pressure it is desirable to allow the excess gas and the volatile by-products of curing to be removed, preferably by bubbling through oil, glycerine or the like, in the open chamber 60. Of course, neck 58 and chamber 60 will not be necessary, when 48' is a vacuum pump. In this manner, it will be understood that the insulated conductor 16' may be provided with a post-curing of the insulation thereon by means of drying oven 14' in a nonoxidizing atmosphere to thereby substantially improve the electrical characteristics of the insulating film.

FIGURE 2a illustrates a modified sealing means which may be used with the curing ovens 14 or 14' of FIGURES 1 and 2, if desired. The modified sealing means of FIGURE 2a is designed for use with a curing oven when the oven is to be used in an evacuated condition. As shown, a sealing member 62 is provided, sealed at its lower end 64 to the drying oven 14. The upper portion of sealing member 62 defines a chamber 66 having upper and lower exits

68, 70, for passage of the conductor 16. Each of exits 68, 70 is sealed by rubber gaskets 72, 74, as shown. A neck member 76 is provided for introducing gas, such as carbon dioxide or nitrogen, into chamber 66 under pressure. A second neck member 78 is provided, leading to open chamber 80 to allow excess gas to be bubbled out through oil or glycerine.

Between exit 70 and sealed end 64 of member 62 is an elongated portion 82, which opens into the curing oven 14. An opening 84 is provided in portion 82 and a neck member 86 extends from such opening. A vacuum pump (not shown) may be secured to neck 86, thus providing for the evacuation of oven 14. It will be understood that the bottom of oven 14 may be sealed in a manner similar to that shown in FIGURES 1 or 2. Alternatively, a sealing means similar to 62 may be provided, if desired. By means of the modified sealing member 62, a vacuum may be drawn within the oven 14, with the blanket of gas in chamber 66 preventing any outside air being drawn through the rubber gaskets, such as 74, into the oven. By use of this modified sealing means a better nonoxidizing atmosphere may be obtained in an evacuated drying oven for use with either the first cure or the post-cure of this invention.

It has been found that various types of insulating enamels which are used for coating electrical conductors may have their electrical properties substantially improved by means of the curing method of this invention. Some types of enamels which have shown special promise in this field are enamels which are made from urea-formaldehydes, epoxies, the polyvinyl formals, and acrylics. Each of these types of enamel insulations has shown marked improvement in their electrical characteristics without deterioration of their physical characteristics when cured according to the method of this invention.

As is well known to those skilled in the electrical insulation art, one measure of the electrical properties of the insulation is the dissipation factor of such insulation. In general, the dissipation factor provides a measure of the electrical resistance of the insulation. As a general rule, the electrical resistance of insulation decreases at increasing temperatures. An increase in the dissipation factor measures the decrease in electrical resistance with an increase in temperature, thus the lower the dissipation factor the better the electrical resistance of the insulation. To provide an indication of the electrical resistance of insulation it is usual to cite the dissipation factor of the insulation at the various temperatures.

FIGURE 3 shows curves which indicate the dissipation factor of various electrical conductors insulated with polyvinyl formal enamel which have been cured in the manner indicated below. The curve of FIG. 3 indicates the dissipation factor of each of these insulations over the various range of temperatures shown in the figure.

For example, considering curve A of FIG. 3 this curve represents polyvinyl formal coated wire which has been cured in an air oven at approximately 250 degrees centigrade for 10 minutes. The wire was provided with (8) coats of the polyvinyl formal enamel, with air curing of each coat. As can be seen by curve A, at 160° the dissipation factor is very low, approximately 7%. However, by the time the temperature reaches approximately 190° C. the dissipation factor of this standard cured polyvinyl formal enamel is approximately 45%. Curve B is the curve of polyvinyl formal enamel coating of (8) coats in which each coat has been cured in a carbon dioxide atmosphere at a temperature of approximately 275° C. for 10 minutes for each coat. As can be seen, the dissipation factor at 160° is slightly lower than that for the standard cured polyvinyl formal enamel insulation, shown in curve A, and at 190° the dissipation factor is approximately 27% indicating an improvement over the regular curing of about 40%.

Curve C is an example of a vacuum cured polyvinyl formal enamel coating which has been subjected to a post-

cure under a vacuum of approximately 8 mm. Hg at 275° C. for approximately 10 minutes. The wire of curve C was provided with (8) coats of polyvinyl formal enamel, with each coat being cured for approximately 10 minutes at 275° C. at a vacuum of 8 to 10 mm. of Hg. When tested at 180° C. this insulated wire had a dissipation factor of approximately 25%, showing only a small improvement over the coated wire of curve A. However, when subjected to post-curing, the electrical properties of this coated wire showed substantial improvement. As can be seen, when the post-cure is provided, a substantial improvement is obtained in the dissipation factor such that at approximately 200° C. the dissipation factor is only approximately 15% and at 220° C. the dissipation factor is less than 30%. Curve D of FIG. 3 is an example of the post-curing under a vacuum of 8 mm. Hg and 275° C. of the polyvinyl formal coated wire of curve B. As can be seen from the curve D, the enamel insulation is very substantially improved by the addition of the post-cure to the previously cured polyvinyl formal under the CO<sub>2</sub> blanket. In this example the dissipation factor at 200° C. is less than 10%, while at 230° C. the dissipation factor is still under 30%. Thus as will be seen from FIG. 3, by means of curing of the polyvinyl formal enamel in a nonoxidizing atmosphere, as disclosed in curve B, a substantial improvement may be obtained in its electrical insulating qualities. However, when an additional post-cure is provided even further substantial improvements are obtained in the electrical insulation properties of the polyvinyl formal coated insulation.

Substantial work has been done in the area of post-curing of various types of enamel insulations which have previously been cured in the normal manner in an air oven. Various types of enamels have been tested in this fashion, and those made from polyesters, epoxies, polyvinyl formals, acrylics and urea-formaldehydes have shown substantial improvement in their electrical properties when subjected to the post-cure of this invention. The following are examples of the types of improvements which have been obtained:

#### Example I

An electrical conductor coated with an acrylic enamel and cured in the standard fashion was subjected to a post-curing at 275° C. for approximately 10 mm. Hg. The dissipation factor of the insulation coating at 130° C. dropped from greater than 50% to approximately 29%.

#### Example II

A standard polyester enamel applied to wire and cured in the normal fashion was found to have a dissipation factor of 50% at 150° C. This wire when treated at 275° C. for approximately 10 minutes at a vacuum of approximately 10 mm. Hg was found to have a dissipation factor of 10% at 190° C. and 28% at 210° C.

#### Example III

An epoxy wire enamel applied to an electrical conductor and cured in the normal manner was found to have a dissipation factor of 42% at 140° C. When this sample was treated at 325° C. for approximately 10 minutes at a vacuum of approximately 10 mm. Hg it was found to have a dissipation factor of 11% at 150° C. and 24% at 160° C. A second sample of this wire was post-cured at 350° C. for approximately 10 minutes in a vacuum of approximately 10 mm. Hg. This second sample was found to have dissipation factor of 11% at 160° C. and 45% at 180° C.

#### Example IV

A wire coated with polyvinyl formal enamel in the usual manner, cured in the usual way was found to have a dissipation factor of 12% at 170° C. and approximately 45% at 190° C. (See curve A, FIGURE 3). One portion of this wire was post-cured at 275° C. for approximately 10 minutes under a vacuum of 10 mm. Hg. This

post-cured wire was found to have a dissipation factor of 7% at 170° C., 22% at 190° C. and 39% at 200° C. A second sample was post-cured at 350° C. for approximately 10 minutes under a vacuum of 10 mm. Hg and was found to have a dissipation factor of only 4% at 170° C., 10% at 190° C. and 33% at 220° C.

*Example V*

A wire conductor was coated with a urea-formaldehyde-phenolic enamel according to standard practice had a dissipation factor of 33% at 160° C. and a 50% dissipation factor at 168° C. This sample was then post-cured at 270° C. for approximately 10 minutes at a vacuum of 10 mm. Hg. After post-curing its dissipation factor was only 3% at 160° C., 12% at 180° C. and did not reach 50% dissipation factor until the temperature was increased to 206° C.

All of the above wire samples were still flexible after the post-curing, as is indicated by a one-time diameter wrap after the post-curing. Thus from the above it is seen that post-curing of various types of electrical insulating enamel will provide a substantial improvement in their electrical properties without any detrimental effects to their physical properties.

Referring now to FIG. 4 of the drawings, there is shown curves indicating the post-cure treatment of polyvinyl formal coated wire according to this invention. Curve A of FIG. 4 is polyvinyl formal coated wire which has been cured in the usual manner. As can be seen, the curve A of FIG. 4 is essentially equivalent to curve A of FIG. 3. Curve B of FIG. 4 is an example of polyvinyl formal coated wire, cured as in curve A, which has been post-cured under a CO<sub>2</sub> atmosphere for approximately 10 minutes at 275° C. As can be seen, the dissipation factor of this insulation is substantially improved over that of curve A. Curve C is another sample of the enamel wire when post-cured at 275° C. for approximately 10 minutes under an N<sub>2</sub> atmosphere. Again, it can be seen that a substantial improvement is obtained in the electrical properties of the insulation when subjected to the post-cure of this invention. Curves D and E are examples of polyvinyl formal coated wire which have been post-cured at approximately 350° C. for 10 minutes, curve D under a vacuum of 8 mm. Hg and curve E under a vacuum of 250 microns of Hg. As can be seen, the improvement in the dissipation factor of these enamels is essentially similar under these vacuum treatment post-cures.

FIGURE 5 shows the curve of a post-cure treatment of an epoxy enamel on an electrical conductor which has been subject to a vacuum curing of approximately 8 mm. Hg for 10 minutes at 275° C. Curve A is the epoxy enamel insulation subject to the normal curing, while curve B is the epoxy enamel insulation subjected to the post-cure of this invention. As can be seen, the epoxy enamel when post-cured according to this invention shows a marked improvement of its electrical properties over the standard cure of curve A.

FIGURE 6 shows the similar results obtained for polyester enamel on an electrical conductor when subjected to a vacuum post-curing of approximately 10 mm. Hg at 275° C. for approximately 10 minutes. As curve A is the polyester enamel with the normal cure, and curve B is the polyester enamel subjected to the post-cure of this invention, again, it is readily apparent the substantial improvement in electrical properties which can be obtained by means of the post-curing of this invention.

In order to further show the substantial improvements which are obtained by the post-curing of this invention, the curves of FIG. 7 have been provided. Curve A of FIG. 7 shows the dissipation factor of polyvinyl formal coated electrical conductors, cured in the usual manner, which have been aged at 175° C. for the days indicated. Curve B is the dissipation factor of polyvinyl formal enamel-insulated electrical conductors which have been post-cured at a vacuum of approximately 8 mm. Hg at

275° C. for 10 minutes. These also are aged at 175° C. for the days indicated. The dissipation factor of the different coils has been determined at 175° C. at the end of the various days. As can be seen, the dissipation factor of the post-cured polyvinyl formal coated coil is substantially lower than that of the normally cured polyvinyl formal enamel and it retains its low dissipation factor for approximately 30 days compared to the approximate 20 days of the standard cured polyvinyl formal enamel coated coils. From this it can be seen that the aging characteristics of the insulating enamel is also substantially improved by means of the post-cure of this invention.

In the various examples set forth above, the various times and temperatures, as well as the nonoxidizing atmosphere have been set forth for various types of enamel coated electrical conductors. From the various information provided it will be apparent that the maximum temperature for post-curing of enamel coated wire will be the temperature at which the particular enamel will decompose. The lower temperatures at which proper post-curing may be obtained will depend greatly upon the type of enamel, the limit of the oven, and the time of travel of the wire through the oven. Obviously, the temperatures must be sufficiently high to obtain a post-cure of the enamel on a dynamic system. Thus the enamel coated wire must run through the oven and the temperatures must be sufficiently high over the period of travel to provide the desired post-cure. For example, as above indicated with polyvinyl formal enamel it is necessary to provide at least 10 minutes of post-cure at 250° C. regardless of the type of nonoxidizing atmosphere. However, where the temperature is raised up to 350° C. for 10 minutes substantially better results are obtained, as has been shown. In a similar fashion, the higher temperatures will in general provide better results, that is, a substantially better increase in the electrical properties of the insulation, as long as the higher temperature does not exceed the temperature at which the particular type of enamel will decompose. In general, it has been found that approximately 10 minutes at this high temperature is sufficient to provide a post-cure which will provide an excellent increase in the electrical properties of the various types of enamel. Of course, with the higher temperatures, substantially improved results may be obtained where the post-cure is less than ten minutes. However, as will be apparent, depending upon the desired properties lower temperatures may be utilized and obviously longer times may be provided in the curing oven to obtain the desired increase in electrical properties. Therefore, while there has been shown and described various preferred embodiments of this invention, and while specific times, temperatures, and types of nonoxidizing atmospheres have been set forth, it will be apparent to those skilled in the art that various changes may be made in the times, temperatures, and atmospheres without departing from the spirit and scope of this invention. The invention to be protected is defined in the following claims.

What is claimed as new and which it is desired to secure by Letters Patent of the United States is:

1. A method of curing a film insulation selected from the group consisting of epoxies, polyesters, acrylics, polyvinyl formals and urea-formaldehydes, in which the film is coated on a conductor and the conductor is heated in a nonoxidizing atmosphere at a temperature below the decomposing temperature of said film insulation said temperature being at least 250° C. for approximately 10 minutes.

2. A method of improving the film insulation on an electrical conductor, where the conductor has a film insulation selected from the group consisting of epoxies, polyesters, acrylics, polyvinyl formals and urea-formaldehydes, comprising the steps of subjecting the insulated conductor to a post-cure in a nonoxidizing atmosphere at a temperature less than the decomposing temperature

of said film insulation said temperature being at least 250° C. for approximately 10 minutes.

3. A method of providing an improved polyvinyl formal film insulation on an electrical conductor comprising the steps of passing the conductor through a bath of liquid polyvinyl formal insulating material, then passing the coated conductor through a curing oven wherein the curing oven is provided with a nonoxidizing atmosphere and in which the curing oven is maintained at a temperature not less than 250° C. and not in excess of 350° C. and each segment of the coated conductor passes through the oven in not more than 10 minutes.

4. A method of providing an improved polyvinyl formal film insulation on an electrical conductor comprising the steps of passing the conductor through a bath of liquid polyvinyl formal insulating material then passing the coated conductor through a curing oven wherein the curing oven is provided with a nonoxidizing atmosphere

and then post curing the insulated conductor in a non-oxidizing atmosphere at a temperature not less than 250° C. and not in excess of the decomposing temperature of the polyvinyl formal insulation for approximately 10 minutes.

## References Cited by the Examiner

## UNITED STATES PATENTS

2,970,936 2/1961 Richardson ----- 117—218 X

## FOREIGN PATENTS

16,338 3/1956 Germany.

730,289 5/1955 Great Britain.

ALFRED L. LEAVITT, Primary Examiner.

WILLIAM L. JARVIS, Examiner.